

April 17, 1934.

D. ADAMS

1,955,163

PROCESS AND APPARATUS FOR ANNEALING SHEET GLASS

Filed July 20, 1931

2 Sheets-Sheet 1



INVENTOR  
Daniel Adams

Frank Fraser

ATTORNEY

April 17, 1934.

D. ADAMS

1,955,163

PROCESS AND APPARATUS FOR ANNEALING SHEET GLASS

Filed July 20, 1931

2 Sheets-Sheet 2



INVENTOR  
Daniel Adams

BY

*Frank Fraser*

ATTORNEY

## UNITED STATES PATENT OFFICE

1,955,163

PROCESS AND APPARATUS FOR ANNEALING  
SHEET GLASSDaniel Adams, Evanston, Ill., assignor to Libbey-  
Owens-Ford Glass Company, Toledo, Ohio, a  
corporation of Ohio

Application July 20, 1931, Serial No. 551,856

24 Claims. (Cl. 49—47)

The present invention relates to an improved process and apparatus for annealing sheet glass or other sheet material.

It is an aim of this invention to provide a novel process and apparatus for annealing sheet glass wherein the said sheets can be thoroughly and uniformly annealed while being passed through an annealing zone or leer at a relatively more rapid speed than heretofore possible.

Another important object of the invention is to provide a process and apparatus wherein the glass sheets are protected against undue loss of heat from the surfaces thereof, whereby to prevent the said surfaces from cooling off in advance of the inner body portion of the sheets, thereby reducing the liability of breakage and the setting up of stresses and strains in the glass during annealing.

A further object of the invention is the provision of a process and apparatus wherein a stream of heated air is caused to flow through the annealing zone or leer in the same direction as the movement of the glass sheets therethrough and in contact with the surfaces thereof, the stream of air at the entrance end of the leer being of substantially the same temperature as that of the sheet as it is passed thereinto, with the said air stream being cooled at the same rate as that of the glass, whereby a uniform annealing of the sheets may be achieved.

Other objects and advantages of the invention will become more apparent during the course of the following description when taken in connection with the accompanying drawings.

In the drawings forming a part of this application and wherein like numerals are employed to designate like parts throughout the same,

Fig. 1 is a vertical longitudinal section through an annealing leer constructed in accordance with the present invention, and

Fig. 2 is a front end view thereof, partially broken away.

Referring now to the drawings in detail, the annealing oven or leer is designated in its entirety by the numeral 5 and, as shown, is of the continuous tunnel type including the top 6, bottom 7, and vertical side walls 8, preferably formed of a suitable refractory material. The leer is also provided with the end walls 9 and 10 which are preferably of metal. The end wall 9 at the entrance end of the leer comprises a plate 11 constituting a closure for the corresponding end of the said leer and having a horizontally disposed slot 12 therein through which the glass sheets 13 may be introduced. Carried upon or formed

integral with the back of plate 11 and disposed vertically at opposite sides of the leer are the conduits 14 in communication with the interior of said leer through the lateral openings 15 and 16 positioned above and beneath the path of travel 60 of the glass sheets 13.

The vertical conduits 14 carried by the closure plate 11 extend downwardly beneath the bottom 7 of the leer as indicated at 17 and 18 and communicate with a casing 19 within which is housed 65 a suitable blower 20, this blower being driven from a motor 21 through reduction gearing located in the gear housing 22. The air being blown upwardly through the conduits 17 and 18 into conduits 14 and thence into the leer is adapted 70 to be heated by means of suitable burners or the like 23.

The end wall 10 for the exit end of the leer is of substantially the same construction as wall 9 and comprises a plate 24 constituting a closure 75 for the corresponding end of said leer and having a horizontal slot 25 therein through which the sheets may be removed. Carried by or formed integral with the back of this plate and arranged at each side of the leer is a vertical conduit 26 80 having lateral openings 27 and 28 communicating with the interior of the leer above and beneath the path of travel of the glass sheets. The vertical conduits 26 carried by closure plate 24 project upwardly beyond the top 6 of the leer as indicated at 29 and 30 and communicate with a casing 31 within which is located a conventional suction device 32 driven from the motor 33 through suitable reduction gearing contained 85 in the housing 34.

The sheets of glass 13 may be supported and conveyed through the leer upon a series of horizontally aligned rolls 35 driven in any desired manner. Arranged within the leer above and beneath rolls 35 are a plurality of spaced transversely extending baffle members or plates 36, said baffle plates being carried by the top and bottom walls 6 and 7 and inclining in the direction of travel of the glass sheets. It is to be noted, however, that the adjacent free ends of the baffle plates are spaced from the glass sheets to provide unrestricted passages at the top and bottom thereof. Positioned between adjacent baffle plates and in relatively close proximity to the top and bottom of the leer and extending transversely thereof are a plurality of pipes 37 through which is adapted to be circulated a suitable cooling medium such as water or the like.

In carrying out the present invention, there is adapted to be passed through the leer 5 in the 110

- same direction as the travel of the glass sheets 13 therethrough and in surrounding relation thereto a heated stream of air which is adapted to assist in the annealing of the glass. This air 5 is forced upwardly by the blower 20 through the conduits 17 and 18 into conduits 14 and thence through openings 15 and 16 into the leer above and beneath the glass sheets. This air is then caused, upon operation of the suction device 32, 10 to travel horizontally through the leer in substantially surrounding relation to the glass sheets and in contact with the surfaces thereof as indicated by the arrows in Fig. 1, the air being drawn outwardly of the leer at the exit end thereof through openings 27 and 28 into conduits 15 26 and thence through conduits 29 and 30. The air being forced into the leer at the entrance end thereof is adapted to be heated by the means 23 to a temperature substantially equal to the temperature 20 of the glass sheets as they enter the leer. For example, assuming the sheet upon entering the leer to be of a temperature of substantially 1500 degrees Fahrenheit, the air being forced into the leer by the blower will also be heated to a temperature of 1500 degrees Fahrenheit. During the flow of the air stream longitudinally through the leer, a suitable cooling medium is adapted to be circulated through the pipes 37, and the metal baffle plates 36 are adapted 25 to pocket air therebetween so as to keep the stream of heated air away from the cold pipes. The glass, however, will lose heat rapidly by radiation to the cold pipes 37 and the air stream will be caused to cool at the same rate as the glass, thereby protecting the glass against undue loss of heat from the surfaces thereof. Inasmuch as the air stream is cooled at the same rate as the glass sheet, it will be of substantially the same temperature as the said sheet when 30 removed from the leer. Thus, if the sheet upon emerging from the leer has a temperature of approximately 200 degrees Fahrenheit, the air being withdrawn will be of substantially the same temperature.
- 45 Due to the provision of the stream of air in surrounding relation to the sheet, and the cooling of this air stream at the same rate as the glass, it will be readily apparent that the glass will be thoroughly and uniformly annealed and 50 that the setting up of stresses and strains therein, which might be caused by a too rapid cooling off of the glass surfaces in advance of the body portion thereof, will be obviated. Moreover, with such an arrangement it is possible to pass the 55 glass sheets through the leer relatively more rapidly than has been heretofore possible.
- It is to be understood that the form of the invention herewith shown and described is to be taken as the preferred embodiment of the same, 60 and that various changes in the shape, size and arrangement of parts may be resorted to without departing from the spirit of the invention or the scope of the subjoined claims.
- I claim:
- 65 1. An annealing leer of the continuous tunnel type, including a series of horizontally arranged rolls for supporting and conveying sheet material to be annealed therethrough, means for effecting the positive movement of a stream of air through 70 the leer from one end thereof to the other above and beneath the sheet material and in contact therewith, and means for heating the air prior to its introduction into said leer.
- 75 2. An annealing leer of the continuous tunnel type, including a series of horizontally arranged rolls for supporting and conveying sheet material to be annealed therethrough, means for setting up a continuous flow of air through the leer in the same direction as the movement of the sheet material therethrough above and beneath the same and in contact therewith, and means for heating the air prior to its introduction into said leer. 80
3. An annealing leer of the continuous tunnel type, including a series of horizontally arranged rolls for supporting and conveying sheet material to be annealed therethrough, means for effecting the positive movement of a stream of air through the leer from one end thereof to the other above and beneath the sheet material and in contact therewith, means for heating the air prior to its entrance into said leer to a temperature substantially equal to the temperature of the sheet material entering the leer, and means for effecting an equal cooling of the air and sheet material as they travel through said leer. 85
4. An annealing leer of the continuous tunnel type, including a series of horizontally arranged rolls for supporting and conveying sheet material to be annealed therethrough, means for setting up a continuous flow of air through the leer in the same direction as the movement of the sheet material therethrough above and beneath the same and in contact therewith, means for heating the air prior to its entrance into said leer to a 100 temperature substantially equal to the temperature of the sheet material entering the leer, and means for effecting an equal cooling of the air and sheet material as they travel through said leer. 105
5. An annealing leer of the continuous tunnel type, including means for supporting and conveying sheet material to be annealed therethrough, mechanical means for effecting the positive movement of a stream of air through the leer in substantially surrounding relation to the sheet material and in contact therewith, means for heating the air prior to its entrance into said leer to a 110 temperature substantially equal to the temperature of the sheet material entering the leer, and means disposed within said leer out of the path of travel of the air and sheet material therethrough for effecting a simultaneous and equal cooling thereof. 115
6. An annealing leer of the continuous tunnel type, including means for supporting and conveying sheet material to be annealed therethrough, mechanical means for setting up a continuous flow of air through the leer in the same direction as the movement of the sheet material therethrough and in contact therewith, means for heating the air prior to its entrance into said leer to a 120 temperature substantially equal to the temperature of the sheet material entering the leer, and means disposed within said leer out of the path of travel of the air and sheet material therethrough for effecting a simultaneous and equal cooling thereof. 125
7. An annealing leer of the continuous tunnel type, including means for supporting and conveying sheet material to be annealed therethrough, mechanical means for effecting the positive movement of a stream of air through the leer in substantially surrounding relation to the sheet material and in contact therewith, means for heating the air prior to its entrance into said leer to a 130 temperature substantially equal to the temperature of the sheet material entering the leer, and a plurality of spaced cooling members extending transversely within said leer above and beneath 135
- 140
- 145
- 150

- the path of travel of the sheet material for effecting a simultaneous and equal cooling of the sheet material and air as they move through the leer.
8. An annealing leer of the continuous tunnel type, including means for supporting and conveying sheet material to be annealed therethrough, mechanical means for setting up a continuous flow of air through the leer in the same direction as the movement of the sheet material therethrough and in contact therewith, means for heating the air prior to its entrance into said leer to a temperature substantially equal to the temperature of the sheet material entering the leer, and a plurality of spaced cooling members extending transversely within said leer above and beneath the path of travel of the sheet material for effecting a simultaneous and equal cooling of the sheet material and air as they move through the leer.
- 10 9. An annealing leer of the continuous tunnel type, including means for supporting and conveying sheet material to be annealed therethrough, mechanical means for effecting the positive movement of a stream of air through the leer in substantially surrounding relation to the sheet material and in contact therewith, means for heating the air prior to its entrance into said leer to a temperature substantially equal to the temperature of the sheet material entering the leer, means for effecting an equal cooling of the air and sheet material as they travel through said leer, and means for preventing the stream of heated air from coming into contact with said cooling means.
- 15 10. An annealing leer of the continuous tunnel type, including means for supporting and conveying sheet material to be annealed therethrough, mechanical means for setting up a continuous flow of air through the leer in the same direction as the movement of the sheet material therethrough and in contact therewith, means for heating the air prior to its entrance into said leer to a temperature substantially equal to the temperature of the sheet material entering the leer, means for effecting an equal cooling of the air and sheet material as they travel through said leer, and means for preventing the flow of heated air from coming into contact with said cooling means.
- 20 11. An annealing leer of the continuous tunnel type, including means for supporting and conveying sheet material to be annealed therethrough, mechanical means for effecting the positive movement of a stream of air through the leer in substantially surrounding relation to the sheet material and in contact therewith, means for heating the air prior to its entrance into said leer to a temperature substantially equal to the temperature of the sheet material entering the leer, means disposed within said leer out of the path of travel of the air and sheet material therethrough for effecting a simultaneous and equal cooling thereof, and a series of baffle members disposed above and beneath the sheet material for pocketing air therebetween to maintain the flow of heated air passing through the leer away from said cooling means.
- 25 12. An annealing leer of the continuous tunnel type, including means for supporting and conveying sheet material to be annealed therethrough, mechanical means for setting up a continuous flow of air through the leer in the same direction as the movement of the sheet material therethrough and in contact therewith, means for heating the air prior to its entrance into said leer to a temperature substantially equal to the temperature of the sheet material entering the leer, means disposed within said leer out of the path of travel of the air and sheet material therethrough for effecting a simultaneous and equal cooling thereof, and a series of baffle members disposed above and beneath the sheet material for pocketing air therebetween to maintain the flow of heated air passing through the leer away from said cooling means.
- 30 13. An annealing leer of the continuous tunnel type, including means for supporting and conveying sheet material to be annealed therethrough and in contact therewith, means for heating the air prior to its entrance into said leer to a temperature substantially equal to the temperature of the sheet material entering the leer, means disposed within said leer out of the path of travel of the air and sheet material therethrough for effecting a simultaneous and equal cooling thereof, and a series of baffle members disposed above and beneath the sheet material for pocketing air therebetween to maintain the flow of heated air passing through the leer away from said cooling means, said baffle members inclining in the direction of travel of the sheet material through said leer.
- 35 14. An annealing leer of the continuous tunnel type, including means for supporting and conveying sheet material to be annealed therethrough, end walls for the leer, each including a plate constituting a closure for the corresponding end of said leer and having a conduit carried thereby and communicating with the leer, means associated with the conduit of the front end wall of the leer for forcing air into said leer, and suction means associated with the conduit of the wall at the exit end of the leer for withdrawing the air therefrom.
- 40 15. An annealing leer of the continuous tunnel type, including means for supporting and conveying sheet material to be annealed therethrough, end walls for the leer, each including a plate constituting a closure for the corresponding end of said leer and having a conduit carried thereby and communicating with the leer, means associated with the conduit of the front end wall of the leer for forcing air into said leer, suction means associated with the conduit of the wall at the exit end of the leer for withdrawing the air therefrom, and means for heating the air prior to its entrance into said leer.
- 45 16. An annealing leer of the continuous tunnel type, including means for supporting and conveying sheet material to be annealed therethrough, end walls for the leer, each including a plate constituting a closure for the corresponding end of said leer and having a conduit carried thereby and communicating with the leer, means associated with the conduit of the front end wall of the leer for forcing air into said leer, suction means associated with the conduit of the wall at the exit end of the leer for withdrawing the air therefrom, means for heating the air prior to its entrance into said leer, and means within the leer for effecting an equal cooling of the heated air and sheet material.
- 50 17. An annealing leer of the continuous tunnel type, including means for supporting and conveying sheet material to be annealed therethrough, end walls for the leer, each including a plate constituting a closure for the corresponding end of said leer and having a conduit carried

- thereby and communicating with the leer, means associated with the conduit of the front end wall of the leer for forcing air into said leer, suction means associated with the conduit of the wall at 5 the exit end of the leer for withdrawing the air therefrom, means for heating the air prior to its entrance into said leer, means within the leer for effecting an equal cooling of the heated air and sheet material, and a plurality of spaced baffle members arranged transversely within the leer for pocketing air therebetween and preventing the heated air from coming into contact with said cooling means.
18. An annealing leer of the continuous tunnel type, including means for supporting and conveying sheet material to be annealed therethrough, end walls for the leer, each including a plate constituting a closure for the corresponding end of the leer and having vertical conduits 15 carried thereby at opposite sides of said leer and communicating therewith through lateral openings above and beneath the path of travel of the sheet material, means associated with the conduits of the front end wall of the leer for forcing air into the said leer, means associated with the conduits of the wall at the exit end of the leer for withdrawing the air therefrom, means for heating the air prior to its entrance into the leer, a plurality of spaced cooling members extending 20 transversely within the leer above and beneath the path of travel of the sheet material and air therethrough, and a plurality of spaced baffle plates also extending transversely within the leer and inclining in the direction of travel of the 25 sheet material therethrough for pocketing air therebetween whereby to prevent the heated air from coming into contact with said cooling members.
19. The process of annealing sheet glass, which 30 consists in carrying the sheet in a definite substantially horizontal path through an annealing chamber on constantly shifting separated lines of transverse support, in setting up the positive movement of a stream of air through said chamber in the same direction as the movement of the sheet therethrough above and beneath the same and in contact therewith, heating the air prior 35 to its entrance into the annealing chamber to a temperature substantially equal to the temperature of the sheet upon entering the chamber, and in effecting a simultaneous and equal cooling of the air and sheet as they travel through said chamber.
20. The process of annealing sheet glass, which 40 consists in carrying the sheet in a definite substantially horizontal path through an annealing chamber on constantly shifting separated lines of transverse support, in setting up the positive movement of a stream of air through said chamber in the same direction as the movement of the sheet therethrough above and beneath the same and in contact therewith, heating the air prior to its entrance into the annealing chamber to a temperature substantially equal to the temperature of the sheet upon entering the chamber, in providing mechanical cooling means 45 within said chamber, causing the glass sheet to lose heat by radiation to said cooling means, and in maintaining the stream of heated air out of direct contact with the cooling means.
21. An annealing leer of the continuous tunnel type including means for supporting and conveying sheet material to be annealed therethrough, means for effecting the positive movement of a stream of air through the leer in the same direction as the movement of the sheet material therethrough above and beneath the same and in contact therewith, means for heating the air prior to its introduction into said leer, and means within the leer for restricting the cross sectional area of the stream of air passing therethrough to less than that of the leer and for maintaining the cross sectional area of the said stream substantially constant throughout the length of said leer. 50
22. An annealing leer of the continuous tunnel type including a series of horizontally arranged rolls for supporting and conveying sheet material to be annealed therethrough, mechanical means for effecting the positive movement of a stream of air through the leer in the same direction as the movement of the sheet material therethrough above and beneath the same and in contact therewith, means for heating the air prior to its introduction into said leer, and a series of baffle members arranged within the leer above and beneath the path of travel of said sheet for restricting the cross sectional area of the stream of air to less than that of the leer and for maintaining the cross sectional area of the said stream substantially constant throughout the length of said leer. 55
23. An annealing leer of the continuous tunnel type including means for supporting and conveying sheet material to be annealed therethrough, mechanical means for effecting the positive movement of a stream of air through the leer in substantially surrounding relation to the sheet material and in contact therewith, means for heating the air prior to its introduction into said leer, and a series of baffle members positioned above and beneath the path of travel of said sheet material, the baffle members in each series being spaced substantially equal distances apart throughout the leer and being of a uniform length. 60
24. An annealing leer of the continuous tunnel type including means for supporting and conveying sheet material to be annealed therethrough, mechanical means for effecting the positive movement of a stream of air through the leer in substantially surrounding relation to the sheet material and in contact therewith, means for heating the air prior to its introduction into said leer, a series of baffle members carried by the top and bottom walls of the leer and positioned above and beneath the path of travel of said sheet material, the baffle members in each series being spaced substantially equal distances apart throughout the leer and being of a uniform length, and a plurality of cooling pipes positioned between adjacent baffle members in relatively close proximity to the top and bottom of the said leer and extending transversely thereof. 65

DANIEL ADAMS.

140